

# United States Patent [19]

Giles et al.

[11] 3,859,079

[45] Jan. 7, 1975

[54] **HIGH TEMPERATURE OXIDATION  
RESISTANT ALLOY**

[75] Inventors: **Philip M. Giles; Arnold R. Marder,**  
both of Bethlehem, Pa.

[73] Assignee: **Bethlehem Steel Corporation,**  
Bethlehem, Pa.

[22] Filed: **Aug. 9, 1972**

[21] Appl. No.: **275,650**

[52] U.S. Cl. .... **75/124, 75/126 D**

[51] Int. Cl. .... **C22c 37/10**

[58] Field of Search ..... **75/124, 126 D**

[56] **References Cited**

UNITED STATES PATENTS

|           |         |                  |        |
|-----------|---------|------------------|--------|
| 1,621,523 | 3/1927  | Clement.....     | 75/124 |
| 1,641,752 | 9/1927  | Flintermann..... | 75/124 |
| 1,833,723 | 11/1931 | Ruder .....      | 75/124 |

|           |         |              |        |
|-----------|---------|--------------|--------|
| 2,941,883 | 6/1960  | Ida.....     | 75/124 |
| 2,987,394 | 6/1961  | Mueller..... | 75/124 |
| 3,068,094 | 12/1962 | Zackay ..... | 75/124 |
| 3,676,109 | 7/1972  | Cooper ..... | 75/124 |

Primary Examiner—Hyland Bizot  
Attorney, Agent, or Firm—Joseph J. O'Keefe; William  
B. Noll

[57] **ABSTRACT**

A low-cost ferrous alloy having improved high-temperature oxidation-resistance under conditions of cyclic heating at temperatures up to about 2500°F, and consisting essentially of, by weight percent, about 4.0 to 8.2% aluminum, up to about 10.5% chromium, about .05 to 2.0% titanium, with the balance iron and incidental impurities, said alloy further characterized by an *f* factor  $\geq 9.0$ , where:

$$f = (\% \text{ Al}) + 0.4(\% \text{ Cr}) + 2.5(\% \text{ Ti}).$$

**3 Claims, 1 Drawing Figure**

PATENTED JAN 7 1975

3,859,079



## HIGH TEMPERATURE OXIDATION RESISTANT ALLOY

### BACKGROUND OF THE INVENTION

This invention relates to a low-cost, high-temperature oxidation-resistant ferrous alloy suitable for applications where thermal shock, such as cyclic heating and cooling, are experienced. While not intending to unduly limit this invention, applications which can take advantage of the properties hereof are high temperature exhaust systems in automobiles, jet engines, and in the petrochemical industry.

Heretofore, high-temperature oxidation-resistant materials were selected from high cost nickel and cobalt superalloys or ceramic materials. In an effort to lower costs, the prior art moved to lower or less rich alloys. For example, U.S. Pat. No. 1,641,752 teaches a ferrous alloy resistant to oxidation at high temperatures, by including therein a high percentage of aluminum. Specifically, said alloy contains from 12 to 20% aluminum, and about 1 to 5% of a grain refining material, among which the patentee has included titanium and chromium. The high temperature oxidation-resistance is due at least in part to the formation of a protective coating of oxide of the aluminum on the exposed surfaces of the ferrous alloy. However, such alloys are of limited suitability under cyclic heating and cooling conditions wherein thermal shock results in flaking and spalling of the oxide coating. Accordingly, one of the critical requirements of a suitable alloy is its ability to resist such flaking and spalling.

### SUMMARY OF THE INVENTION

The present invention relates to a ferrous alloy which is not only resistant to oxidation at high temperatures, but is resistant to surface flaking and spalling when subjected to thermal shocking as a result of cyclic heating and cooling. More particularly, said invention covers an element balanced alloy consisting essentially of, by weight percent, about 4.0 to 8.2% aluminum, up to about 10.5% chromium, about 0.05 to 2.0% titanium, with the balance iron and incidental impurities. Further, the element balancing is achieved by the formula:  $f = (\% \text{ Al}) + 0.4(\% \text{ Cr}) + 2.5(\% \text{ Ti})$ , where the value of  $f$  is at least 9.0

### BRIEF DESCRIPTION OF DRAWINGS

The FIGURE is a graph of time of exposure to failure vs.  $f$  for a series of ferrous alloys falling within the alloying ranges noted previously, with time plotted on a logarithmic scale.

### DETAILED DESCRIPTION OF PREFERRED EMBODIMENT

This invention relates to an oxidation resistant ferrous alloy, more particularly to a wrought ferrous alloy suitable for use in applications where ability to withstand thermal shock is critical. Typical applications where the latter characteristic is significant are high temperature exhaust systems, such as a thermal reactor in automobiles, jet engines, and in the petrochemical industry. While the mention of same is not intended as a limitation on this invention, it is believed that a brief discussion thereof will help in understanding the significance of this invention and the contributions offered thereby.

Generally, a thermal reactor is a container into which the hot exhaust gases flow from the automotive, jet or power producing engines, for further combustion. Air is also pumped into the reactor and admixed with said gases. The reactor is generally of sufficient size (chamber volume) to give a long enough residence time of the admixed gases to permit complete combustion of the residual hydrocarbons and carbon monoxide. Since the combustion reaction is so strongly exothermic, temperatures may go as high as 2200°F., typically about 1800°F., in a highly oxidizing environment. Thus, the severe conditions of high temperature, oxidizing environment, and intermittent operation (cyclic heating and cooling), call for a material capable of meeting these conditions. The alloys of the present invention not only fulfill these conditions, but accomplish it at a low material cost.

The composition of the alloys of this invention fall broadly within the alloying ranges below:

|          |   |                  |
|----------|---|------------------|
| Aluminum | — | 4.0 to 8.2 wt. % |
| Titanium | — | .05 to 2.0 wt. % |
| Chromium | — | up to 10.5 wt. % |
| Carbon   | — | up to 0.10 wt. % |
| Iron     | — | balance,         |

except that within said ranges the composition must satisfy the formula,  $f = (\% \text{ Al}) + 0.4(\% \text{ Cr}) + 2.5(\% \text{ Ti}) \geq 9$ , and the titanium content must exceed 4 times the carbon content. A preferred composition is one containing at least 5.0% chromium, aluminum between about 6.0 to 8.0% and titanium between about 0.4 to 1.10%.

While no maximum value for  $f$  has been noted, if desirable one can readily be calculated from the richest composition contained within the limits above. However, it is believed that such a figure would not be significant as to the alloy's performance under severe oxidizing conditions. The maximum composition limits, and hence the maximum  $f$ , are established by other considerations, such as material cost and processing restrictions.

In this regard, the production of wrought strip and sheet by conventional rolling practices requires that the material be sufficiently ductile for said rolling to be effected. In the case of aluminum containing iron base alloys, the ductility thereof drops below a practical level when the aluminum begins to exceed about 8% by weight. Chromium, when added to an Al-Fe alloy, should not exceed about 10% by weight, as the risk of breakage and other processing problems increases. Finally, with respect to carbon it should be kept to a low value, preferably less than about 0.04% typically less than 0.03%. But in no case should it exceed 25% of the titanium.

It should be apparent by this time that the significant features of this invention are achieved by a proper balance of the alloy's composition such that the value of  $f$ , heretofore defined, exceeds about 9.0. With such an alloy, it will be observed that upon exposing said alloy to a highly oxidizing atmosphere at high temperatures, there develops an adherent oxide coating. This coating is predominantly oxides of aluminum, titanium and combinations thereof, with little or no iron oxide. This iron oxide free coating resists flaking, spalling and thermal shock so as to protect the alloy from catastrophic oxidation. As used herein, catastrophic oxidation is the presence of black oxide coating in an amount greater

than 30% of the surface area exposed to the oxidizing atmosphere.

The very adherent oxide coating which forms on the alloy of this invention must contain some oxides of titanium. Thus, while it may not be apparent at this juncture, the titanium forms a dual function. The carbon in an alloy of the type described herein tends to migrate to the grain boundaries as carbides. By adding titanium, a strong carbide former, the carbon is readily tied up as titanium carbide and is uniformly dispersed throughout the alloy. Thus, sufficient titanium must be present to handle the carbon as well as to be free to assist in forming the adherent oxide coating which resists spalling and flaking. The significance of the titanium is clearly illustrated in the data to follow.

To demonstrate the effectiveness of the ferrous alloys of this invention to resist oxidation at high temperature, attention is directed to the following table and accompanying FIGURE, which dramatically illustrate the superior results achieved in balancing the composition thereof, so as to reflect a value for *f* of at least 9.0.

TABLE

| Sample * | C    | Al   | Cr    | Ti   | "f"   | Time-to-Failure<br>(Hours) at<br>2200° F. |
|----------|------|------|-------|------|-------|-------------------------------------------|
| A        | .009 | 4.20 | —     | —    | 4.20  | .5                                        |
| B        | .015 | 4.04 | —     | .25  | 4.67  | .5                                        |
| C        | .012 | 6.00 | —     | —    | 6.00  | 23                                        |
| D        | .004 | 4.11 | 5.03  | —    | 6.13  | 23                                        |
| E        | .003 | 4.07 | 4.97  | .28  | 6.76  | 23                                        |
| F        | .015 | 4.02 | —     | 1.10 | 6.77  | .5                                        |
| G        | .020 | 5.02 | 4.96  | —    | 7.00  | 23                                        |
| H        | .016 | 5.98 | —     | .54  | 7.33  | 23                                        |
| J        | .019 | 4.93 | 4.94  | .25  | 7.52  | 47                                        |
| K        | .022 | 4.01 | 9.66  | —    | 7.87  | 23                                        |
| L        | .009 | 8.12 | —     | —    | 8.12  | 63                                        |
| M        | .008 | 8.10 | —     | .28  | 8.80  | 1087                                      |
| N        | .013 | 8.00 | —     | .52  | 9.30  | 1771                                      |
| P        | .037 | 6.92 | 3.08  | .53  | 9.46  | 1565                                      |
| Q        | .016 | 5.97 | 9.74  | —    | 9.87  | 111                                       |
| R        | .019 | 7.92 | 5.00  | —    | 9.92  | 229                                       |
| S        | .015 | 8.01 | —     | 1.02 | 10.56 | 2631                                      |
| T        | .016 | 5.92 | 9.75  | .49  | 11.04 | 2998                                      |
| U        | .007 | 6.18 | 10.32 | .53  | 11.63 | >3300                                     |

where:  $f = (\% \text{ wt Al} + .4 (\% \text{ wt Cr} + 2.5 (\% \text{ wt Ti}))$

\* Mo, P, S, Sn<0.1% Cu, Mn, V<0.02% Ni<0.03%

The procedure used to determine time-to-failure at 2200°F. was as follows:

The samples, nominally 1 inch  $\times$  2 inches  $\times$  0.050 inch, were hung on silicon carbide bars using chromel wire through a hole drilled in one end thereof. The bars were then placed in an exposed-element, electrically heated furnace at  $2200^\circ \pm 20^\circ \text{ F}$ . Twice daily, the silicon carbide bars with the samples attached were removed from the furnace where the samples were allowed to air cool in still air for about 20 minutes at which time the temperature had dropped to about 200°F. The samples were then returned to the furnace. The long term average cycle time was about 15 hours.

The samples were periodically inspected and considered to have failed when either about 30% of the sample surface was covered with a porous black oxide, or when the area around the hole oxidized to the point of actually failing or by their appearance being unable to support the weight any further.

In any case, by these objective standards, it is readily apparent from the tabular and graphic data that a significant improvement resulted when the composition of 10 the alloy was balanced to an *f* value of about 9.0, and titanium was present in an amount of at least 0.05%. Note specifically samples Q and R where *f* exceeded 9.0 but the titanium was lacking. A comparison of Samples Q and T, whose difference is essentially the addition of about 0.49% Ti, shows nearly a thirteen (13) fold improvement in oxidation resistance with said titanium.

We claim:

1. A ferrous alloy resistant to catastrophic oxidation under conditions of repeated cyclic heating and cooling between the temperatures of 2,200° F. and 200° F., said

ferrous alloy composed of, by weight percent, a maximum of 0.04% carbon, aluminum between about 4.0 and 8.2%, chromium up to about 10.5%, titanium between 0.4 and 1.10%; and the balance substantially iron, except that said ferrous alloy is characterized by a value of *f* of at least about 9.0, where:

$$f = (\% \text{ Al}) + 0.4(\% \text{ Cr}) + 2.5(\% \text{ Ti}), \text{ and } (\% \text{ Ti}) > 4(\% \text{ C}).$$

55 2. The alloy claimed in claim 1 wherein said chromium is present in an amount of at least 5.0%.

3. The alloy claimed in claim 1 wherein said aluminum is present in an amount between about 6.0 and 8.0%.

\* \* \* \* \*